

## UNITED STATES PATENT OFFICE.

ROBERT H. LEACH, OF BRIDGEPORT, CONNECTICUT, ASSIGNOR TO HANDY & HARMEN,  
A CORPORATION OF NEW YORK.

## SILVER ALLOY.

No Drawing.

Application filed August 25, 1923. Serial No. 659,394.

This invention relates to an improvement in silver alloys, and the object of the invention is to provide a silver which has great resistance to tarnishing or other discoloration, or more specifically the object embraces an alloy containing a preponderating amount of silver and also containing cadmium and antimony.

This alloy is to be made preferably of 10 sterling fineness, and the term "sterling" is used to designate a silver alloy which contains, per thousand parts, approximately 925 parts of silver and 75 parts of base metal, which is usually copper. Such silver is subject to discoloration and this may result either by reason of various substances contained in dilute form in the atmosphere, or, in the case of table ware, the discoloration or tarnish may result from the exposure of 20 the metal to the action of fruit acids, foods containing sulphur in various forms, and other substances which contain elements which act on the silver.

As has previously been stated, it is the 25 object of this invention to provide a silver, preferably of sterling quality, which resists discoloration, and I accomplish this result by substituting for the copper ordinarily used in such an alloy, cadmium and antimony. Such an alloy not only resists tarnishing but by the proper selection of the proportions of these metals an alloy may be produced which has varying mechanical qualities.

33 It has been found that when cadmium is added to silver there is produced a very ductile white alloy which can be worked by rolling, spinning, and the like, to a greater extent than the standard silver-copper alloy, 40 without becoming hard. The cadmium appears to form a homogeneous alloy which is of uniform quality and which is satisfactory in many respects as, for instance, having tarnish resisting properties, but such an 45 alloy is usually so soft that an article made from it, provided little work is done on the metal during the manufacture, will be comparatively soft and will not offer sufficient resistance to ordinary use. Such an article 50 will, therefore, become dented or bent readily, and is objectionable for that reason.

On the other hand, the addition of antimony to a silver alloy increases the resistance of the metal to tarnish, and in addition 55 makes it quite brittle and difficult to work.

However, by combining the three ingredients above mentioned, namely, silver, antimony and cadmium, in proper proportions, it is possible to secure an alloy which has the desired tarnish-resisting qualities and which has the ductility, and malleability which may be required for any particular use.

An alloy which fulfills the above requirements will contain a preponderating amount of silver, for instance, about 92.5%, when 65 the alloy is to be of sterling fineness, and an amount of cadmium varying between 1% and 7%, and antimony between 6.5% and 0.5%. An alloy in which the cadmium approaches the upper limit will be comparatively soft and ductile, and will be used for the production of articles in which considerable working of the metal is required, while where little working is carried on during the manufacture, the alloy will contain 75 cadmium approaching the lower limit. For what may be called a general purpose alloy, the proportions will be approximately 2.5% of cadmium and 5% of antimony, the remainder of the alloy being made up of 80 92.5% of silver, when the alloy is to be of sterling quality.

From a scientific viewpoint a silver alloy which is designated as solid may contain as low as 66 2/3% of silver, the remainder being 85 made up of various base metals with copper usually employed heretofore.

Silver which is used for manufacturing purposes may also run as high as 95% pure silver, in which event it is, of course, finer 90 than sterling. That silver which is in greatest demand is sterling silver, and I have previously described the proportions of the ingredients which will be present in my non-tarnishing alloy of that fineness, 95 but it is to be understood that by following the principles of the invention here set forth, it is possible to make alloys of other than sterling fineness which will have qualities which will be required by the purposes to 100 which the alloy is to be put. As I have stated, cadmium with silver produces a ductile alloy which has tarnish-resisting properties, but this alloy is so soft that unless some hardening ingredient is employed an 105 article made from such a combination would be easily dented and bent. Accordingly, antimony is employed and the addition of the antimony makes it possible to control the malleability and ductility. The amount of 110

antimony which will be included will naturally be selected in accordance with the purpose to which the alloy is to be put, but it may be said, in general, that the cadmium present will range from about 13% to about 93% of the combined amount of cadmium and antimony present, while the antimony will consequently range from about 87% to about 7% of this combined amount. The skilled metallurgist will be able to determine without difficulty the amount of antimony which is to be included in order to secure a metal of the desired mechanical qualities.

In producing such an alloy various methods may be used, but one convenient method consists in first making up an alloy of silver and cadmium which contains approximately 60% of silver and 40% of cadmium. The cadmium is first melted in a reducing atmosphere under a heavy protective cover such as charcoal, then the silver separately melted and preferably under a cover, is added thereto and the two metals thoroughly mixed. A sample of this mixture which is found to be very homogeneous, is taken and analyzed and on the basis of this analysis there is computed the necessary amount of fine silver and antimony which is required to make the final mixture. The silver which is to be added is then melted and after it is thoroughly liquid the required amount of antimony is added thereto to form a silver-antimony mixture. To this molten mixture the proper weight of the silver-cadmium alloy is added, and with this method the metals are found to be mingled in the final product in a uniform manner. These several melting and mixing steps should be carried on in a reducing atmosphere to secure the best results.

While the above process is entirely sat-

isfactory I do not desire to limit myself to this exact procedure. In any process, however, for the production of this alloy, care should be taken in the manner in which the cadmium is added, inasmuch as it is readily oxidized at the temperature at which the melting is carried on.

An alloy containing the ingredients above referred to is found to resist corrosion or discoloration to a much greater extent than is the case with ordinary alloys containing copper as the base metal. The new alloy, aside from its non-tarnishing qualities, may be made with varying mechanical properties such as hardness, brittleness, and the like, by the proper selection of the amounts of cadmium and antimony used. The antimony combined with the silver not only serves to give the silver a tarnish-resisting quality but also serves to harden the alloy. In view of the properties possessed by the new alloy, it will be apparent that it is capable of wide use in the production of various metallic articles and is desirable for the manufacture of table ware or hollow ware.

I claim:

1. An alloy containing a preponderating amount of silver and about 7.5% of cadmium and antimony, the cadmium ranging from about 1% to 7% and the antimony from about 6.5% to 0.5%.

2. An alloy containing about 92.5% of silver and about 7.5% of cadmium and antimony, the cadmium ranging from about 1% to 7%, and the antimony from about 6.5% to 0.5%.

3. An alloy containing about 925 parts of silver, about 50 parts of antimony, and about 25 parts of cadmium.

In testimony whereof I affix my signature.

ROBERT H. LEACH.

antimony which will be included will naturally be selected in accordance with the purpose to which the alloy is to be put, but it may be said, in general, that the cadmium 5 present will range from about 13% to about 93% of the combined amount of cadmium and antimony present, while the antimony will consequently range from about 87% to about 7% of this combined amount. The 10 skilled metallurgist will be able to determine without difficulty the amount of antimony which is to be included in order to secure a metal of the desired mechanical qualities.

15 In producing such an alloy various methods may be used, but one convenient method consists in first making up an alloy of silver and cadmium which contains approximately 60% of silver and 40% of cadmium. The 20 cadmium is first melted in a reducing atmosphere under a heavy protective cover such as charcoal, then the silver separately melted and preferably under a cover, is added thereto and the two metals thoroughly mixed. A 25 sample of this mixture which is found to be very homogeneous, is taken and analyzed and on the basis of this analysis there is computed the necessary amount of fine silver and antimony which is required to make the 30 final mixture. The silver which is to be added is then melted and after it is thoroughly liquid the required amount of antimony is added thereto to form a silver-antimony mixture. To this molten mixture 35 the proper weight of the silver-cadmium alloy is added, and with this method the metals are found to be mingled in the final product in a uniform manner. These several melting and mixing steps should be carried on 40 in a reducing atmosphere to secure the best results.

While the above process is entirely sat-

isfactory I do not desire to limit myself to this exact procedure. In any process, however, for the production of this alloy, care 45 should be taken in the manner in which the cadmium is added, inasmuch as it is readily oxidized at the temperature at which the melting is carried on.

An alloy containing the ingredients above 50 referred to is found to resist corrosion or discoloration to a much greater extent than is the case with ordinary alloys containing copper as the base metal. The new alloy, aside from its non-tarnishing qualities, may 55 be made with varying mechanical properties such as hardness, brittleness, and the like, by the proper selection of the amounts of cadmium and antimony used. The antimony combined with the silver not only serves to 60 give the silver a tarnish-resisting quality but also serves to harden the alloy. In view of the properties possessed by the new alloy, it will be apparent that it is capable of wide 65 use in the production of various metallic articles and is desirable for the manufacture of table ware or hollow ware.

I claim:

1. An alloy containing a preponderating amount of silver and about 7.5% of cadmium 70 and antimony, the cadmium ranging from about 1% to 7% and the antimony from about 6.5% to 0.5%.

2. An alloy containing about 92.5% of silver and about 7.5% of cadmium and anti- 75 mony, the cadmium ranging from about 1% to 7%, and the antimony from about 6.5% to 0.5%.

3. An alloy containing about 925 parts of silver, about 50 parts of antimony, and about 80 25 parts of cadmium.

In testimony whereof I affix my signature.

ROBERT H. LEACH.

#### CERTIFICATE OF CORRECTION.

Patent No. 1,628,673.

Granted May 17, 1927, to

ROBERT H. LEACH.

It is hereby certified that the name of the second mentioned assignee in the above numbered patent was erroneously written and printed as "Harmen" whereas said name should have been written and printed as "Harman", as shown by the records of assignments in this office; and that the said Letters Patent should be read with this correction therein that the same may conform to the record of the case in the Patent Office.

Signed and sealed this 7th day of June, A. D. 1927.

Seal.

M. J. Moore,  
Acting Commissioner of Patents.

CERTIFICATE OF CORRECTION.

Patent No. 1,628,673.

Granted May 17, 1927, to

ROBERT H. LEACH.

It is hereby certified that the name of the second mentioned assignee in the above numbered patent was erroneously written and printed as "Harmen" whereas said name should have been written and printed as "Harman", as shown by the records of assignments in this office; and that the said Letters Patent should be read with this correction therein that the same may conform to the record of the case in the Patent Office.

Signed and sealed this 7th day of June, A. D. 1927.

Seal.

M. J. Moore,  
Acting Commissioner of Patents.